

Oct. 3, 1933.

C. P. LEYNER ET AL  
METHOD OF FINISHING SURFACES OF MATERIALS  
COMPOSED IN PART OF VEGETABLE FIBERS  
Filed June 23, 1932

1,929,117



Fig. 1.



Fig. 2.



Fig. 4.



Fig. 3.



Fig. 5.

Inventors

Charles P. Leyner,  
Rosa M. Leyner.

By *A. J. O'Brien*  
Attorney

## UNITED STATES PATENT OFFICE

1,929,117

## METHOD OF FINISHING SURFACES OF MATERIALS COMPOSED IN PART OF VEGETABLE FIBERS

Charles P. Leyner and Rosa M. Leyner, Denver,  
Colo.

Application June 23, 1932. Serial No. 618,856

6 Claims. (Cl. 92—68)

This invention relates to improvements in methods for surfacing fiber boards of the type that are made from compressed vegetable fibers.

In the erection of buildings it is getting quite customary to employ fiber boards of different type like those made from sugarcane bagasse, corn stalk, wood fiber, etc.

Fiber boards of the type referred to are very good insulators against heat and cold and are also poor conductors of sound vibration and are therefore admirably suited for building construction. In many places the inner walls composed of fiber board are left exposed and unfinished for different reasons, and when this is the case it is desirable to give them a finish that will produce a pleasing and ornamental appearance and for this purpose we have invented a method of finishing the surface of fiber boards that will impart to these surfaces a peculiar finish that improves the appearance and also has a very beneficial and desirable effect in connection with sound reflection and which make the fiber boards thus finished especially well adapted for use in rooms devoted to radio broadcasting or the testing of musical instruments, radios, etc.

This invention, briefly described, consists in subjecting the surface of the fiber board to the action of a coarse abrasive, such as coarse sand or carborundum paper or to the action of a rotating abrasive wheel made of carborundum or some equivalent abrasive. The effect of subjecting the surfaces to the action of an abrasive is to release the ends of the vegetable fibers and remove from the same the pulp that adheres to them so as to produce a nap which, when the abrasive is moved in one direction only during the operation, produces a nap that is composed of the vegetable fibers which extend in substantially the same direction and give to the surface a velvety finish with a silky appearance.

The napped surface that is produced by the method which forms the subject of this invention not only improves the appearance, but as above intimated, has a very important effect in connection with sound reflection because it appears that when sound waves strike the velvety nap, they are not reflected to any appreciable extent, whereas, if the surface is left hard and smooth as it is with the original finish, then the sound reflections are greatly increased.

In addition to improving the appearance and the sound reflecting characteristics of the fiber boards by the process which will be herein described, this process also facilitates the orna-

mentation of tiles and mouldings made from this kind of material.

It has been found that where rotary cutters employing blades, such as are used in connection with the manufacture of wooden mouldings and similar wooden building material are employed in connection with fiber boards the resultant finish is objectionable because it is hard and glossy and is therefore a good reflector for sound waves and at the same time it does not have the finished appearance that similar articles have when made in accordance with the process herein to be described.

Having thus briefly described the invention and some of its advantages, it will now be described in greater detail and for this reason reference will be had to the accompanying drawing in which the invention has been illustrated in such a way that the process and the resultant product can be clearly defined and in which:

Fig. 1 is a plan view of a rectangular tile that is ornamented in a certain way by means of the process herein described;

Fig. 2 shows one form of moulding that has been made by means of an apparatus carrying out the process;

Fig. 3 is a diagrammatic side elevation of a portion of an apparatus employed in carrying out this process;

Fig. 4 is a section through one of the depressions cut by the abrading wheel and shows the nap that is produced by this process; and

Fig. 5 is a section to an enlarged scale and is intended to illustrate the nap produced by the operation of this process.

In the drawing numeral 6 represents a rectangular piece of fiber board of the type referred to in the above parts of the specification, whose surface has been ornamented by having radially extending depressions 7 cut in its surface. These depressions are cut by means of a rotating wheel 8 provided with a cutting surface 9 made of carborundum or some similar coarse grained abrasive. In Fig. 3 the support for the block has been indicated by reference numeral 10 while the fiber that is operated on has been indicated by reference numeral 11. The groove that is cut by the wheel and which corresponds to the one indicated by numeral 7 in Fig. 1 has been designated by reference numeral 12. The machine shown is merely a diagrammatic representation of a machine that can be used for this purpose and consists of a stationary frame member 13 that has rotatably secured to it a shaft 14 which carries a belt wheel 15. A link 16 has its

upper end pivoted to the shaft 14 and its lower end pivotally connected at 17 with the frame 18 to which the wheel 8 is journaled. Two belt wheels which are represented by reference 5 numeral 19 are pivoted on the shaft 17 and a belt wheel 20 is connected to the shaft 21 that carries the wheel 8. When shaft 14 is rotated by a motor, the wheel 8 will rotate in the direction of the arrow and by moving the frame forwardly 10 while the wheel is rotating the surface of the fiber will be abraded so as to leave a nap 22 composed of the outer ends of the vegetable fibers which the action of the abradant has cleaned and separated from each other and laid in one direction 15 so that the surface resembles the surface of velvet.

Although in the examples illustrated the surface has been acted upon by means of a wheel that changes the formation of the surface so as 20 to produce lines or curved effects as in the moulding it is to be understood that the surface can be processed in the manner described without ornamenting the same and when this is done a room that is finished by means of fiber board 25 subjected to treatment like the one described will give an appearance resembling that which would be obtained by having a velvet covering of the same color.

Attention is called to the fact that the fiber 30 boards that are employed for this purpose can be dyed so as to give any colored effect desired without interfering with the proper functioning of the nap in the prevention of sound reflection.

From the above it will be apparent that we 35 have produced an improved method for finishing the surface of boards composed principally of vegetable fibers which not only improves the appearance, but also alters the characteristics of the surface in regard to sound reflection and which 40 also prevents the reflection of light to a great

extent and therefore makes the surface especially well adapted for use in rooms where optical tests are being conducted and where it is desired to obviate the glare that is usually produced by smooth hard finished surfaces.

Having described the invention what is claimed as new is:

1. The method of ornamenting the surfaces of boards containing vegetable fibers which consists in subjecting the surface of the board to the action of an abrasive member and thereby producing designs in intaglio whose surfaces are covered with a nap comprising the ends of fibers. 80

2. The method of producing ornamental designs in intaglio in articles made from vegetable fiber which consists in grinding depressed areas by the action of an abrasive member, whereby designs in intaglio are produced and whereby the surfaces of the designs are given a velvety finish. 90

3. The herein described method of ornamenting the surface of material composed of vegetable fibers consisting in removing a portion of said material to produce designs in intaglio. 95

4. The herein described method of ornamenting the surface of material composed of vegetable fibers consisting in removing said material by a grinding action to produce designs in intaglio. 100

5. The herein described method of ornamenting the surface of material composed of vegetable fibers consisting in removing a portion of said material by an abrasive action to produce designs in intaglio. 105

6. The herein described method of ornamenting the surface of material composed of vegetable fibers consisting in removing a portion of said material by a rotary abrasive action to produce designs in intaglio. 110

CHARLES P. LEYNER.  
ROSA M. LEYNER.

115

45

120

50

125

55

130

60

135

65

140

70

145

75

150